# EUROPEAN PATENT SPECIFICATION

(11) **EP 1 482 061 B1**
(45) Date of publication and mention of the grant of the patent: **11.05.2011**
(21) Application number: 03703098.8
(22) Date of filing: 30.01.2003
(51) Int. Cl.: C22B 1/248, C22B 1/243

(54) **BRITTLE MOLDED ARTICLE AND BRIQUETTE USING THE SAME**
SPRÖDER FORMKÖRPER UND BRIKETT, BEI DEM DIESER VERWENDET WIRD
ARTICLE MOULE FRAGILE ET BRIQUETTE ASSOCIEE

(30) Priority: 31.01.2002 JP 2002023804
(43) Date of publication of application: 01.12.2004
(73) Proprietor: JTEKT Corporation, Osaka-shi Osaka 542-8502 (JP)
(72) Inventor: MATSUDA, Mitsuma, Kagawa-gun, Kagawa-ken 761-1702 (JP); SEDOU, Masafumi, KOBE-SHI, Hyogo 658-0065 (JP)
(74) Representative: Sajda, Wolf E.
(86) International application number: PCT/JP2003/000945
(87) International publication number: WO 2003/064709

(56) References cited:
- EP-A- 1 323 838
- DE-A1- 4 432 721
- GB-A- 1 301 235
- JP-A- 7 116 960
- JP-A- 9 256 078
- JP-A- 51 103 003
- JP-A- 53 010 563
- JP-A- 2002 194 449
- US-A- 4 585 475
- PATENT ABSTRACTS OF JAPAN vol. 1998, no. 01, 30 January 1998 (1998-01-30) & JP 09 256078 A (NISSHIN STEEL CO LTD; IWAKUNI SEISAKUSHO:KK), 30 September 1997 (1997-09-30)

## Description

### TECHNICAL FIELD

The present invention relates to a dried briquette comprising powdered pure iron and oil, and a method of forming such a briquette.

### BACKGROUND ART

Shavings produced when grinding (hereinafter this term is used as a concept including polishing, super finishing polishing, lapping and so on) a ferrous metal such as quenched bearing steel or carburized steel are recovered as a flocculent (fibrous) agglomerate containing abrasive grains, a grinding liquid containing water and oil, and so on. Such a flocculent agglomerate contains a large amount of pure iron, and attempts have been made to reuse this as a steel-making raw material. However, the flocculent agglomerate contains a large amount of water, and hence if the flocculent agglomerate is put into a blast furnace as is, then due to the water a problem of bumping (steam explosion) occurring will be brought about. One can thus envisage removing the water from out of the flocculent agglomerate by centrifugation or the like. In this case, the oil contained in the flocculent agglomerate will be removed together with the water, and hence the pure iron that is a component of the shavings will be changed into iron oxide due to self heating of the flocculent agglomerate. In this case, reduction is thus necessary to enable reuse as a steel-making raw material, and the cost increases due to the use of a reducing agent and so on.

Moreover, shavings having the above-mentioned oil attached thereto do not readily stick together, and hence if a flocculent agglomerate is compression molded as is then it will be difficult to solidify the flocculent agglomerate to the desired strength. Furthermore, for a flocculent agglomerate containing a large amount of ferrous metal shavings having a carbon content of at least 0.2 wt%, there will be much spring-back upon compression, and hence even if such a flocculent agglomerate is compression molded it will be difficult to solidify the flocculent agglomerate to the desired strength. Consequently, if the compression molded flocculent agglomerate is put into a blast furnace, then a problem will arise in that the flocculent agglomerate will fly up and scatter around, and hence the majority will be collected by a dust collector.

Furthermore, pulverization of the fibrous shavings contained in a flocculent agglomerate as described above is difficult using a hammer mill or the like, and hence the flocculent agglomerate cannot be finely sheared. It is thus also difficult to process such a flocculent agglomerate into briquettes or the like.

The actual state of affairs is thus that a flocculent agglomerate as described above is not reused, but rather is consigned to a waste disposal company and disposed of as landfill.

However, such disposal of the flocculent agglomerate as landfill is undesirable from the viewpoint of the effective utilization of resources. Moreover, there are problems of deterioration of the environment being brought about, and the disposal cost being high.

The document EP-A-1 323 838 which is to be considered under Article 54(3) EPC discloses a dried briquette comprising powdered pure iron and oil, wherein the briquette is a brittle molded body, obtained by compression molding a fibrous agglomerate comprising ferrous metal shavings and a grinding liquid containing oil and water, thereby shearing to solidify the shavings into the brittle molded body, wherein the brittle molded body is strengthened with a solidification assistant impregnated therein, wherein the solidification assistant is at least one selected from colloidal silica, sodium silicate, aluminum phosphate, and emulsified asphalt. Also, a method of forming such a briquette is disclosed in this context. The document is silent, however, as to any bulk specific gravity values of the briquette and any percentages of fibrous agglomerate of unquenched ferrous metal in the briquette.

The document JP-A-09-256 078 discloses a formed material which can be suitable for use for deoiling by heating under reduced pressure. For this purpose, the conventional formed material has an almost columnar shape which is produced by compress-forming metallic scraps with a forming device. The prior art does not discuss any materials to be added as solidification assistants or any amounts of such solidification assistants to be impregnated in order to form the molded bodies.

The document GB-A-1 301 235 discloses a method for shaft furnace smelting of oxidic materials which comprises the steps of heating the oxidic materials at a suitable temperature, blending the hot calcines with carbonaceous fuel reductant containing a caking component to form a hot mixture in which heat is transferred to the carbonaceous fuel reductant from the hot calcine, briquetting the hot mixture, and subjecting the briquettes to shaft furnace smelting. Further features of the conventional method relate to specific materials, like flux matieral and caking coal as well as specific temperatures used in the method. The document is silent, however, as to the use of any specific solidification assistants, the amount of such solidification assistants to be impregnated and any structure which may have a softer core and a strengthened layer on the outer surface side thereof.

The object underlying the present invention is to provide a dried briquette comprising powdered pure iron and oil, as well as a method of forming such a briquette, in which ferrous metal shavings can efficiently be reused so that such briquettes can readily be used for steel making.

According to the invention, the object is solved by means of a dried briquette comprising powdered pure iron and oil, wherein the briquette is a brittle molded body, obtained by compression molding a fibrous agglomerate comprising ferrous metal shavings and a grinding liquid containing oil and water, thereby shearing to solidify the shavings into the brittle molded body, wherein the fibrous agglomerate includes 30 to 50 wt% of fibrous agglomerate of unquenched ferrous metal so that the obtained brittle molded body has a bulk specific gravity of 3.0 to 4.5, wherein on the surface side a strengthened layer is formed of a higher bulk specific gravity by not less than 0.5 and higher hardness than on the inner side, wherein the brittle molded body is strengthened with a solidification assistant impregnated therein and contained in an amount of 2 to 30 wt%, and wherein the solidification assistant is at least one selected from colloidal silica, sodium silicate, aluminum phosphate, and emulsified asphalt.

Advantageous further developments of the dried briquette according to the invention are specified in the sub-claims.

As to the method, the object is solved by a method of forming a briquette comprising the following steps:
- compression molding into a prescribed shape a fibrous agglomerate comprising ferrous metal shavings and a grinding liquid containing oil and water, thereby shearing the shavings, wherein a fibrous agglomerate is used which includes 30 to 50 wt% of fibrous agglomerate of unquenched ferrous metal to form a porous brittle molded body having a bulk specific gravity of 3.0 to 4.5 and having a strengthened layer on a surface side of the brittle molded body;
   impregnating the obtained brittle molded body with a solidification assistant to make the solidification assistant penetrate into the brittle molded body and strengthen the brittle molded body,
   wherein the solidification assistant is at least one selected from colloidal silica, sodium silicate, aluminum phosphate, and emulsified asphalt, and wherein the brittle molded body contains 2 to 30 wt% of the solidification assistant; and
- drying the brittle molded body impregnated with the solidification assistant to cause the solidification assistant that has penetrated into the inside of the brittle molded body to move to the surface side, thereby further strengthening the strengthened layer.

Advantageous further developments of the method according to the invention are specified in the sub-claims.

With the dried briquette having the constitution as defined according to the invention, the desired strength and shape maintainability can be secured, and handling such as transportation is thus easy. Moreover, because a large amount of pure iron is contained, for example reuse as a material for a high-quality steel-making raw material briquette or a material for sintered metal is possible, and hence the briquette is useful in environmental conservation, and moreover the disposal cost for shavings can be reduced.

When the fibrous agglomerate is obtained by mixing a fibrous agglomerate containing quenched ferrous metal shavings with a fibrous agglomerate containing unquenched ferrous metal shavings, the dried briquette can easily be solidified, and the strength of such briquettes can be further increased.

When the briquette has an oil content of 1 to 12 wt%, the briquette will be solidified to a suitable hardness, and at the same time, oxidation of pure iron, which is a component of the shavings, can effectively be prevented by the small amount of oil.

The briquettes according to the invention have a suitable strength and are not prone to breakage so that handling during transportation, storage and the like is easy. Hence, such briquettes are suitable for steel making. Even if they are put, for example, into a blast furnace, there will be no risk of bumping or of matter flying up since the briquettes have a suitable strength. Since the briquettes contain oil, oxidation of the powdered pure iron is prevented, and such briquettes can suitably be used as a steel raw material in practice.

### BRIEF DESCRIPTION OF THE DRAWINGS

FIG. 1 is a perspective view showing a brittle molded body according to an embodiment of the present invention.
FIG. 2 is a schematic view showing a cross section of the brittle molded body.
FIG. 3 is a graph showing the compressive fracture strength of brittle molded bodies.
FIG. 4 is a process drawing showing a method of manufacturing a brittle molded body and a briquette.

### BEST MODE FOR CARRING OUT THE INVENTION

Following is a detailed description of embodiments of the present invention, with reference to the attached drawings.

FIG. 1 is a perspective view showing a brittle molded body Z according to an embodiment of the present invention. The brittle molded body Z is obtained by solidifying by compression molding into a cylindrical shape a flocculent agglomerate C (see FIG. 4) comprising a grinding liquid containing oil and water and shavings produced when grinding a quenched ferrous metal.

The brittle molded body Z is compression molded such that the bulk specific gravity thereof becomes at least 1.5; as a result, the fibrous shavings are sheared, and a porous brittle body having a suitable amount of oil and voids is formed. Moreover, the oil content of the brittle molded body Z is adjusted to 1 to 12 wt%.

Furthermore, on the surface side of the brittle molded body Z is formed a strengthened layer K of higher density and higher hardness than on the inner side (see FIG. 2). In the case, for example, that the brittle molded body Z is a cylindrical shape with a diameter of 60 to 70 mm and a height of 30 to 40 mm, this strengthened layer K is formed over a region up to a depth of 0.3 to 7.0 mm from the surface; the durometer hardness A in the strengthened layer K is at least 90, and is at least 10 to 30 harder than the durometer hardness A around the central part, and the bulk specific gravity is at least 0.5 to 1 higher than the bulk specific gravity around the central part.

With the brittle molded body Z, oxidation of pure iron that is a component of the shavings is prevented by the residual oil. Moreover, because the bulk specific gravity is at least 1.5 and a strengthened layer K is formed on the surface side, the desired strength and shape maintainability can be secured. Disintegration is thus not prone to occurring when handling during transportation and the like. Furthermore, because the oil content of the brittle molded body Z is 1 to 12 wt%, the brittle molded body Z is solidified to a suitable hardness, and moreover oxidation of the pure iron that is a component of the shavings is prevented effectively by the small amount of residual oil.

As the above-mentioned ferrous metal, one containing at least 0.2 wt% of carbon may be used. Shavings of such a ferrous metal have much spring-back, and hence solidification is difficult, but by using compression molding, the influence of spring-back can be eliminated, and the shavings can be sheared effectively, and hence solidification becomes possible. A representative example of the shavings containing at least 0.2 wt% of carbon is bearing steel shavings.

The brittle molded body Z can be suitably used as, for example, a steel raw material briquette B (see FIG. 4(g)) by impregnating a solidification aid D into the brittle molded body Z to strengthen the brittle molded body Z. As the solidification aid D, it is preferable to use at least one selected from colloidal silica, sodium silicate, aluminum phosphate, and emulsified asphalt, whereby the briquette B can be made stronger despite containing oil. Moreover, the content of the solidification aid D is preferably 2 to 30 wt%, whereby the briquette B can be made yet stronger. Note that vinyl acetate or the like can also be used as the solidification aid D.

With the briquette B, because the brittle molded body Z is further strengthened with the solidification aid D, the briquette B becomes strong, with breakage being less prone to occur when handling during transportation, storage and so on. In particular, because the bulk specific gravity of the brittle molded body Z is at least 1.5, and the strengthened layer K part on the surface side of the brittle molded body Z is effectively solidified by the solidification aid D, the briquette B becomes yet stronger, with breakage being yet less prone to occur. Moreover, because the brittle molded body Z is a porous body having a bulk specific gravity of at least 1.5, and hence the solidification aid D can be made to penetrate deep thereinside with no impediment, the strength of the inside of the briquette B can also be increased effectively. As a result, even if breakage should occur, there will be no risk of the inside part scattering into a powder. Moreover, the briquette B is a dried solid, and hence even if put, for example, into a blast furnace, there will be no risk of bumping occurring or of matter flying up. Furthermore, because the briquette B contains oil, oxidation of the powdered pure iron is prevented. The briquette B is thus particularly suitable as a steel-making raw material briquette.

FIG. 3 is a graph showing the results of carrying out compressive fracture tests on brittle molded bodies and briquettes having different specific gravities. The brittle molded bodies and briquettes used in these compressive fracture tests had a cylindrical shape with an outside diameter of 6.6 cm and a width of 3.5 cm, and the bulk specific gravity was in a range of 1.3 to 2.5 for the brittle molded bodies, and 1.5 to 2.8 for the briquettes. Moreover, the brittle molded bodies were manufactured using flocculent agglomerates obtained by grinding a quenched ferrous metal. The solidification aid impregnated into the brittle molded bodies to obtain the briquettes was an aqueous solution containing approximately 10 wt% of sodium silicate, and this aqueous solution was impregnated into each brittle molded body in an amount of approximately 20% of the volume of the brittle molded body. For the compressive fracture tests, pressure was applied in the radial direction to two opposite points on the outer periphery, and the load upon fracture was measured. The loading rate was set to 1 mm/min.

As is clear from FIG. 3, it was found that the compressive fracture load for brittle molded bodies having a bulk specific gravity of less than 1.5 is less than 150 N and hence these brittle molded bodies are very brittle, whereas the compressive fracture load for brittle molded bodies having a bulk specific gravity of at least 1.5 is in a range of 240 N to 1600 N, i.e. fracture does not readily occur. Moreover, it was found that the fracture strength for the briquettes is 2900 to 4200 N, i.e. a good strength can be secured. In particular, the compressive fracture load required of a steel-making briquette is approximately 2000 N or more, and it was found that this compressive fracture load can be sufficiently secured.

Note that for a flocculent agglomerate C produced when grinding a quenched ferrous metal, depending on the material thereof compression molding may be difficult, but in this case by mixing the flocculent agglomerate C with a flocculent agglomerate C produced when grinding an unquenched ferrous metal, compression molding can be carried out easily and a strong molded body can be obtained. The flocculent agglomerate C of the unquenched ferrous metal is preferably mixed in in an amount of 30 to 50 wt%, whereby a very high-density high-strength brittle molded body Z having a bulk specific gravity of 3.0 to 4.5 and a fracture strength of 2000 to 3000 N can be obtained. Moreover, by impregnating a solidification aid D into this brittle molded body Z, a briquette B having a fracture strength of at least 3100 N can be obtained.

FIG. 4 is a process drawing showing an example of a method of manufacturing a brittle molded body Z and a briquette B as described above. In the manufacture of the brittle molded body Z, first a flocculent agglomerate C of shavings (see FIG. 4(a)) is compressed through application of pressure, thus preliminarily adjusting the contents of water and oil that are components of the grinding liquid contained in the flocculent agglomerate C. The compression of the flocculent agglomerate C through application of pressure is carried out, for example, by conveying the flocculent agglomerate C along a belt conveyor 1 and passing the flocculent agglomerate C between a pair of rollers 2 (see FIG. 4(b)). Note, however, that for the adjustment of the water content and oil content, there are also a method in which this is carried out merely through air blowing or air compression, and a method in which a magnetic separator is used. Here, it is preferable to adjust the water content of the flocculent agglomerate C to a range not exceeding 50 wt%, and the oil content to a range not exceeding 50 wt%. As a result, handling such as transportation and storage of the flocculent agglomerate C becomes easy.

Next, the flocculent agglomerate C for which the water content and the oil content have been adjusted is subjected to compression molding using a molding die 3, e.g. a hydraulic press, thus obtaining a brittle molded body Z (see FIG. 4(c)). Here, the flocculent agglomerate C is compressed such that the bulk specific gravity of the brittle molded body Z becomes at least 1.5. Through the compression molding, spiral fibrous shavings contained in the flocculent agglomerate C are sheared, and moreover a strengthened layer K is formed on the surface side. Moreover, the rate of compression of the flocculent agglomerate C, the water drainage amount and the oil drainage amount during the compression and so on are controlled such that the water content becomes 2 to 12 wt%, and the oil content becomes 1 to 12 wt%. At this time, because the water content and the oil content of the flocculent agglomerate C were each adjusted in advance to a range not exceeding 50 wt% in the previous step, the water content and the oil content in the brittle molded body Z can be adjusted easily and properly.

Next, a liquid solidification aid D is impregnated into the brittle molded body Z. The impregnation of the solidification aid D is carried out, for example, by conveying the brittle molded body Z along a belt conveyor 7 and immersing the brittle molded body Z in the solidification aid D which has been poured into a tank 8 (see FIG. 4(d)).

After that, the brittle molded body Z that has been impregnated with the solidification aid D (see FIG. 4(e)) is cured (dried) (see FIG. 4(f)), whereby a briquette B can be obtained (see FIG. 4(g)). Through the curing, excess solidification aid D that has penetrated to the inside of the brittle molded body Z moves to the surface side, and some of the solidification aid D evaporates, and the remainder remains in the high-density strengthened layer K part, and hence the strengthened layer K part is effectively strengthened.

The brittle molded body Z obtained as described above always retains some of the oil of the grinding liquid including during the processing, and hence oxidation of pure iron that is a component of the shavings is prevented effectively. Moreover, the briquette B is manufactured with some of the oil of the grinding liquid always retained, and hence oxidation of the pure iron is prevented effectively. For example, it was found that a briquette B manufactured using a flocculent agglomerate C containing bearing steel (SUJ-2) shavings contains at least 70 wt% of pure iron. The melting yield is thus very high at at least 70%, and hence the briquettes B can be sold to a steel maker as a high-quality steel-making raw material.

Moreover, with the method of manufacturing the briquette B described above, the flocculent agglomerate C can be solidified without a step of finely pulverizing the flocculent agglomerate C being required, and hence the briquette B can be manufactured efficiently.

Note that when the solidification aid D is impregnated into the brittle molded body Z, the solidification aid D may be diluted with water, a solvent or the like; in this case, the solidification aid D can be made to penetrate deep into the brittle molded body Z more easily and swiftly, and moreover for a solidification aid D containing silicon such as sodium silicate, the amount of silicon can be reduced through the dilution, and hence the amount of impurities is further reduced, which is more preferable as a steel-making raw material.

Moreover, the brittle molded body Z is formed in a shape for which handling is easy, for example the cylindrical shape described above, or a spherical shape, a prismatic shape or the like.

Furthermore, the brittle molded body Z of the present invention may be finely pulverized, whereby instead of reuse as a steel-making raw material briquette B as described above, reuse is possible as a powdered raw material for sintered metal, or an additive in a resin or the like for a magnetic material.

## Claims

1. A dried briquette comprising powdered pure iron and oil,
wherein the briquette is a brittle molded body (Z), obtained by compression molding a fibrous agglomerate (C) comprising ferrous metal shavings and a grinding liquid containing oil and water, thereby shearing to solidify the shavings into the brittle molded body (Z),
wherein the fibrous agglomerate includes 30 to 50 wt% of fibrous agglomerate of unquenched ferrous metal so that the obtained brittle molded body (Z) has a bulk specific gravity of 3.0 to 4.5,
wherein on the surface side a strengthened layer (K) is formed of a higher bulk specific gravity by not less than 0.5 and higher hardness than on the inner side, wherein the brittle molded body (Z) is strengthened with a solidification assistant (D) impregnated therein and contained in an amount of 2 to 30 wt%, and
wherein the solidification assistant (D) is at least one selected from colloidal silica, sodium silicate, aluminum phosphate, and emulsified asphalt.

2. The briquette according to claim 1,
wherein the fibrous agglomerate (C) is obtained by mixing a fibrous agglomerate containing quenched ferrous metal shavings with a fibrous agglomerate (C) containing unquenched ferrous metal shavings.

3. The briquette according to claim 2,
wherein an amount of 30 to 50 wt% of the fibrous agglomerate (C) containing unquenched ferrous metal shavings is mixed into the brittle molded body (Z).

4. The briquette according to any of claims 1 to 3,
having an oil content of 1 to 12 wt%.

5. The briquette according to any of claims 1 to 4,
wherein the ferrous metal contains at least 0.2 wt% of carbon.

6. A method of forming a briquette comprising the following steps:
- compression molding into a prescribed shape a fibrous agglomerate comprising ferrous metal shavings and a grinding liquid containing oil and water, thereby shearing the shavings, wherein a fibrous agglomerate is used which includes 30 to 50 wt% of fibrous agglomerate of unquenched ferrous metal to form a porous brittle molded body (Z) having a bulk specific gravity of 3.0 to 4.5 and having a strengthened layer (K) on a surface side of the brittle molded body (Z);
- impregnating the obtained brittle molded body (Z) with a solidification assistant (D) to make the solidification assistant (D) penetrate into the brittle molded body (Z) and strengthen the brittle molded body (Z),
wherein the solidification assistant (D) is at least one selected from colloidal silica, sodium silicate, aluminum phosphate, and emulsified asphalt, and wherein the brittle molded body (Z) contains 2 to 30 wt% of the solidification assistant (D); and
- drying the brittle molded body (Z) impregnated with the solidification assistant (D) to cause the solidification assistant (D) that has penetrated into the inside of the brittle molded body (Z) to move to the surface side, thereby further strengthening the strengthened layer (K).

7. The method according to claim 6,
wherein the oil content of the brittle molded body (Z) formed by compression molding is adjusted to an oil content of 1 to 12 wt%.

8. The method according to claim 6 or 7,
wherein the hardness of the strengthened layer is adjusted so that the durometer hardness is at least 90, and is at least 10 to 30 harder than the durometer hardness around a central part of the brittle molded body (Z).

## Patentansprüche

1. Getrocknetes Brikett, das pulverförmiges Reineisen und Öl aufweist, wobei es sich bei dem Brikett um einen spröden Formkörper (Z) handelt, der durch Formpressen eines faserigen Agglomerats (C) gebildet ist, das Eisenmetallspäne und eine Öl und Wasser enthaltende Schleifflüssigkeit aufweist, so daß die Späne zerkleinert werden, um diese zu dem spröden Formkörper (Z) zu verfestigen,
wobei das faserige Agglomerat 30 bis 50 Gew.-% faseriges Agglomerat aus nicht abgeschrecktem Eisenmetall enthält, so daß der gebildete spröde Formkörper (Z) eine relative Dichte von 3,0 bis 4,5 aufweist,
wobei an der Oberflächenseite eine verstärkte Schicht (K) mit einer um nicht weniger als 0,5 höheren relativen Dichte und mit einer höheren Härte als an der Innenseite gebildet ist,
wobei der spröde Formkörper (Z) mit einem Verfestigungs-Hilfsmittel (D) verstärkt ist, das darin imprägniert und in einer Menge von 2 bis 30 Gew.-% enthalten ist, und
wobei es sich bei dem Verfestigungs-Hilfsmittel (D) um mindestens eines handelt, das aus kolloidialem Siliziumoxid, Natriumsilikat, Aluminiumphosphat und emulgiertem Asphalt ausgewählt ist.

2. Brikett nach Anspruch 1,
wobei das faserige Agglomerat (C) gebildet ist durch Mischen eines faserigen Agglomerats, das Späne aus abgeschrecktem Eisenmetall enthält, mit einem faserigen Agglomerat (C), das Späne aus nicht abgeschrecktem Eisenmetall enthält.

3. Brikett nach Anspruch 2,
wobei eine Menge von 30 bis 50 Gew.-% des faserigen Agglomerats (C), das Späne aus nicht abgeschrecktem Eisenmetall enthält, in den spröden Formkörper (Z) gemischt ist.

4. Brikett nach einem der Ansprüche 1 bis 3,
der einen Ölgehalt von 1 bis 12 Gew.-% aufweist.

5. Brikett nach einem der Ansprüche 1 bis 4,
wobei das Eisenmetall mindestens 0,2 Gew.-% Kohlenstoff enthält.

6. Verfahren zum Formen eines Briketts,
wobei das Verfahren folgende Schritte aufweist:
- Formpressen eines faserigen Agglomerats, das Eisenmetallspäne und eine Öl und Wasser enthaltende Schleifflüssigkeit aufweist, in eine vorbestimmte Formgebung, um **dadurch** die Späne zu zerkleinern, wobei ein faseriges Agglomerat verwendet wird, das 30 bis 50 Gew.-% faseriges Agglomerat aus nicht abgeschrecktem Eisenmetall enthält, um einen porösen spröden Formkörper (Z) zu bilden, der eine relative Dichte von 3,0 bis 4,5 hat und eine verstärkte Schicht (K) an einer Oberflächenseite des spröden Formkörpers (Z) aufweist;
- Imprägnieren des gebildeten spröden Formkörpers (Z) mit einem Verfestigungs-Hilfsmittel (D), damit das Verstärkungs-Hilfsmittel (D) in den spröden Formkörper (Z) eindringt und den spröden Formkörper (Z) verstärkt, wobei es sich bei dem Verfestigungs-Hilfsmittel (D) um mindestens eines handelt, das aus kolloidialem Siliziumoxid, Natriumsilikat, Aluminiumphosphat und emulgiertem Asphalt ausgewählt wird und wobei der spröde Formkörper (Z) einen Anteil von 2 bis 30 Gew.-% des Verfestigungs-Hilfsmittels enthält; und
- Trocknen des mit dem Verfestigungs-Hilfsmittel (D) imprägnierten spröden Formkörpers (Z), um das in das Innere des spröden Formkörpers (Z) eingedrungene Verfestigungs-Hilfsmittel (D) zu veranlassen, sich an die Oberflächenseite zu bewegen, um **dadurch** die verstärkte Schicht (K) weiter zu verstärken.

7. Verfahren nach Anspruch 6,
wobei der Ölgehalt des durch Formpressen gebildeten spröden Formkörpers (Z) auf einen Ölgehalt von 1 bis 12 Gew.-% eingestellt wird.

8. Verfahren nach Anspruch 6 oder 7,
wobei die Härte der verstärkten Schicht derart eingestellt wird, daß die Durometer-Härte mindestens 90 beträgt und mindestens 10 bis 30 härter ist als die Durometer-Härte um einen zentralen Bereich des spröden Formkörpers (Z).

## Revendications

1. Briquette séchée comprenant du fer pur en poudre et de l'huile, laquelle briquette est un corps moulé cassant (Z), obtenu par moulage par compression d'un agglomérat fibreux (C) comprenant des copeaux de métal ferreux et un liquide de broyage contenant de l'huile et de l'eau, réalisant ainsi un cisaillement pour solidifier les copeaux dans le corps moulé cassant (Z),
dans laquelle l'agglomérat fibreux contient 30 à 50 % en poids d'agglomérat fibreux d'un métal ferreux non trempé de façon que le corps moulé cassant obtenu (Z) ait une densité apparente de 3,0 à 4,5,
dans laquelle, sur le côté de surface, une couche renforcée (K) est formée avec une densité apparente non inférieure à 0,5 et une dureté supérieure à celle du côté intérieur,
dans laquelle le corps moulé cassant (Z) est renforcé avec un auxiliaire de solidification (D) imprégné dans celui-ci et présent en une quantité de 2 à 30 % en poids, et
dans laquelle l'auxiliaire de solidification (D) est au moins un composé choisi parmi la silice colloïdale, le silicate de sodium, le phosphate d'aluminium, et l'asphalte émulsionné.

2. Briquette selon la revendication 1,
dans laquelle l'agglomérat fibreux (C) est obtenu par mélange d'un agglomérat fibreux contenant des copeaux de métal ferreux trempé avec un agglomérat fibreux (C) contenant des copeaux de métal ferreux non trempé.

3. Briquette selon la revendication 2,
dans laquelle une quantité de 30 à 50 % en poids de l'agglomérat fibreux (C) contenant des copeaux de métal ferreux non trempé est mélangée dans le corps moulé cassant (Z).

4. Briquette selon l'une quelconque des revendications 1 à 3,
ayant une teneur en huile de 1 à 12 % en poids.

5. Briquette selon l'une quelconque des revendications 1 à 4,
dans laquelle le métal ferreux contient au moins 0,2 % en poids de carbone.

6. Procédé pour former une briquette, comprenant les étapes suivantes:
- moulage par compression en une forme prescrite d'un agglomérat fibreux comprenant des copeaux de métal ferreux et un liquide de broyage contenant de l'huile et de l'eau, réalisant ainsi un cisaillement des copeaux, étant utilisé un agglomérat fibreux contenant 30 à 50 % en poids d'agglomérat fibreux d'un métal ferreux non trempé pour former un corps moulé cassant poreux (Z) ayant une densité apparente de 3,0 à 4,5 et ayant une couche renforcée (K) sur un côté de surface du corps moulé cassant (Z);
- imprégnation du corps moulé cassant obtenu (Z) avec un auxiliaire de solidification (D) pour que l'auxiliaire de solidification (D) pénètre dans le corps moulé cassant (Z) et renforce le corps moulé cassant (Z), l'auxiliaire de solidification (D) étant au moins un composé choisi parmi la silice colloïdale, le silicate de sodium, le phosphate d'aluminium, et l'asphalte émulsionné, et le corps moulé cassant (Z) contenant 2 à 30 % en poids de l'auxiliaire de solidification (D); et
- séchage du corps moulé cassant (Z) imprégné de l'auxiliaire de solidification (D) pour faire en sorte que l'auxiliaire de solidification (D) qui a pénétré dans l'intérieur du corps moulé cassant (Z) se déplace vers le côté de surface, en renforçant ainsi davantage la couche renforcée (K).

7. Procédé selon la revendication 6,
dans lequel la teneur en huile du corps moulé cassant (Z) formé par moulage par compression est ajustée à une teneur en huile de 1 à 12 % en poids.

8. Procédé selon la revendication 6 ou 7,
dans lequel la dureté de la couche renforcée est ajustée de façon que la dureté au duromètre soit d'au moins 90, et soit plus dure d'au moins 10 à 30 points que la dureté au duromètre autour d'une partie centrale du corps moulé cassant (Z).
